

W. H. WAGGAMAN, C. R. WAGNER & H. BRYAN.  
PROCESS FOR THE MANUFACTURE OF PHOSPHORUS, PHOSPHORIC ACID, &c.  
APPLICATION FILED NOV. 12, 1917.

1,282,994.

Patented Oct. 29, 1918.



*Inventors,*  
William H. Waggamman,  
Cary R. Wagner,  
Harry Bryan,  
By W. M. C. Morris,  
Solicitor,  
Attorney for Applicants.

# UNITED STATES PATENT OFFICE.

WILLIAM H. WAGGAMAN, CARY R. WAGNER, AND HARRY BRYAN, OF WASHINGTON,  
DISTRICT OF COLUMBIA.

## PROCESS FOR THE MANUFACTURE OF PHOSPHORUS, PHOSPHORIC ACID, &c.

1,282,994.

Specification of Letters Patent. Patented Oct. 29, 1918.

Application filed November 12, 1917. Serial No. 201,634.

(DEDICATED TO THE PUBLIC.)

*To all whom it may concern:*

Be it known that we, WILLIAM H. WAGGAMAN, CARY R. WAGNER, and HARRY BRYAN, all citizens of the United States and employees of the Department of Agriculture of the United States of America, residing in the District of Columbia, (whose post-office address is Washington, District of Columbia,) have invented a new and useful Process for the Manufacture of Phosphorus, Phosphoric Acid, and Compounds of the Same.

This application is made under the act of March 3, 1883, chapter 143 (22 Stat., 625), and the invention herein described and claimed may be used by the Government of the United States or any of its officers or employees in the prosecution of work for the Government, or any person in the United States, without payment of any royalty thereon.

Our invention relates to a process for making phosphorus, phosphoric acid, and compounds of the same, and has for its object the production of such products and compounds more expeditiously and economically than heretofore.

With these and other objects in view the invention consists in the novel combination of agents and procedures as will be more fully hereinafter disclosed and particularly pointed out in the claims. This process is designed to be used in an apparatus having the main features of that described in United States Patent No. 1,241,791, issued jointly to us under date of October 2, 1917.

In order that the precise invention may be more clearly understood and distinguished from the prior art, it is said: It is a well-known fact that phosphorus and phosphoric acid can be volatilized from its compounds by submitting an intimate mixture of coke, silicious material and the phosphate material to the action of a high heat. It is generally believed, however, that the complete or nearly complete evolution of the phosphorus or phosphoric acid cannot be effected except at the high temperatures attainable only in an electric furnace. Since the electrical heating of low-grade materials and the recovery thereby of relatively low-priced products may in some instances be commercially impracticable, it is highly

desirable that such material be handled in a furnace where the cost of making the desired product is much cheaper than in an electric furnace. Although it has been stated that phosphorus and phosphoric acid can be only partially freed from their compounds in a fuel-fed furnace of the ordinary blast furnace type, the inventors have found that ninety per cent. or more of these materials can be volatilized from mixtures of phosphate rock, silica and coke at temperatures far below those attained in a blast furnace, and concluded therefore that it was only necessary to employ a modified type of furnace and adjust the working conditions in order to obtain a high yield of phosphoric acid by means of fuel either contained in or intimately mixed with the charge and burned by means of air blasts, or introduced independent of the charge and burned by means of air or oxygen in any well known manner, the heat produced being transferred to the charge causing the evolution of phosphorus or phosphoric acid from their compounds.

The furnace designed for this purpose and described in detail in Patent No. 1,241,791 is of such a type that the phosphorus and phosphoric acid may be driven off as soon as they are freed from their compounds and led out of the reaction zone without being forced to pass through a column of green charge which is often composed of such finely divided material as to offer considerable resistance to the passage of the gases of combustion and volatilized products.

The accompanying drawing forming a part of this specification shows a vertical sectional view of the apparatus built to carry out our invention. The charging bell 1 is of the conventional design ordinarily employed for blast furnaces. The chamber 2 is built of or lined with some refractory material 3 into which the proper proportions of materials for the smelting operation are charged. This chamber is constricted at 3' in order that the charge may not work down through the shaft too rapidly. The lower end of the charge chamber 2, is some distance above the hearth or base of the furnace, the walls 3 of said chamber being supported on the arches or piers 4. The platform 5 receives the materials as they are continuously discharged from the cham-

ber 2. The burners 6 supply heat to the furnace. Said burners may be for oil, coal, gas or any other well known fuel. The flame from said burners plays upon the partially fused material on the platform 5. The slag thus formed runs off the platform onto the hearth 7 and is withdrawn from time to time, through the tap hole 8. Surrounding the charge chamber 2 is the fume chamber 10 into which rise the volatile products of the reactions taking place on the platform 5. Finally the volatilized products are withdrawn through the exit pipe 10 in the upper part of the chamber 9.

15 The process of operating consists in allowing the charge of phosphate, silicious material and coke to feed down through an inner or charge chamber upon a table where it is heated by means of burning fuel, such 20 fuel being either mixed with the charge or introduced from an outside source. The products of combustion and the volatilized products are then led out through a chamber surrounding the charge chamber and the 25 phosphorus and phosphoric acid recovered in some suitable manner.

Having thus described our invention, we claim:

1. The process of obtaining phosphorus or 30 its compounds from mineral phosphate-containing material which comprises mixing such material with silica and carbonaceous

matter, feeding a column of the mixture to a zone of combustion, maintaining a temperature of incandescence in said zone of combustion, passing the products of combustion around the oncoming charge but out of contact therewith whereby the charge is preheated but no phosphorus is deposited therein and collecting phosphorus compounds 40 from the volatile products.

2. The process of obtaining phosphorus or its compounds from mineral phosphate-containing material which comprises mixing such material with silica and carbonaceous matter, feeding a column of such charge into a heated zone while maintaining a temperature of incandescence in said zone by the combustion therein of fuel, passing the products of combustion around the incoming charge but out of contact therewith, whereby the charge is preheated but no phosphorus is deposited therein and collecting phosphorus compounds from the volatile products, substantially as described. 50

In testimony whereof, we affix our signatures in the presence of two subscribing witnesses.

WILLIAM H. WAGGAMAN.  
CARY R. WAGNER.  
HARRY BRYAN.

Witnesses:

J. P. SCHROEDER.  
T. R. LE COMPTÉ.